

1

3,576,629

DIFFUSION TRANSFER MATERIALS AND PROCESS WITH DERIVATIVES OF 4-AMINO-1,2,4-TRIAZOLINE-5-THIONE AS TONING AGENTS  
Kiyoshi Futaki and Noboru Itoh, Kyoto, Sendgi Tosa, Osaka, and Hirokazu Tsukahara, Kyoto, Japan, assignors to Mitsubishi Paper Mills, Ltd., Tokyo, Japan  
No Drawing. Filed Mar. 11, 1968, Ser. No. 711,880  
Claims priority, application Japan, Mar. 27, 1967,

42/18,646

Int. Cl. G03c 5/54

U.S. Cl. 96—29

5 Claims

## ABSTRACT OF THE DISCLOSURE

A diffusion transfer image having densely black image tone is produced by effecting development and diffusion in the presence of 4-amino-1,2,4-triazoline-5-thione derivatives. The examples of said derivatives are 4-amino-3-ethyl-1,2,4-triazoline-5-thione, 4-amino-3-propyl-1,2,4-triazoline-5-thione, etc.

This invention relates to an improved photographic silver complex diffusion transfer process for obtaining diffusion transfer images possessing a densely black image tone and a developer and a photographic material used for said process.

The principle of the silver complex diffusion transfer process can be briefly described as follows: a light-sensitive silver halide emulsion layer which is coated on a base-sheet such as paper or plastic film is imagewise exposed and thereupon pressed into contact with an image-receiving layer which is coated with colloidal dispersion of a heavy metal or metal sulfide immersed in a hydrophilic binder such as gelatin or polyvinyl-alcohol, in the presence of a developing agent and a complexing agent for silver halide. The exposed silver halide grains are developed to metallic silver images and do not undergo any further change, while the unexposed part of the light-sensitive layer is complexed with a complexing agent such as a thiosulfate, a sulfite or an organic amine which is present either in the developer or in the image-receiving layer, where it is converted into metallic silver image by means of colloidal metallic particles which act as developing nuclei during development. In such a way, a positive image of the original appears in the image receiving layer after separating the latter from the light-sensitive layer.

One of the most serious defects of the silver complex diffusion transfer processes in the early stage of progress of this process is the disagreeable brown or yellowish image-tone of the final positive images, and it was necessary to use a gold- or selenium toning to change the color to neutral-black or pleasant sepia-black by after-treatments, and recently it was found that the introduction of some sorts of substance such as mercapto-benzothiazole, benzotriazole, phenyl-mercapto-tetrazole, usually known as antifogging or blue-black toner in an usual photographic silver halide emulsion layer, could also change the tone of image-color of a receiving layer from brown to neutral or blue-black.

These organic heterocyclic compounds, however, usually make sparingly soluble complexes with silver halide and accordingly tend to decrease both the rate of development in an sensitive layer and the rate of image-formation in a receiving layer, and it was difficult to obtain a useful or-

2

ganic toner which does not prolong the developing and transfer time and makes neutral black image of sufficiently density.

And it was a usual practice to combine these developing-retarding blue-black toners such as benzotriazole, 5-nitro-benzimidazole or phenyl-mercapto-tetrazole with some of the substances which are known as an accelerator for developer, such as benzylamine,  $\beta$ -phenyl-ethylamine and N-dodecylpyridinium salt, because these accelerators usually have not effect or sometimes adverse effects on the image color.

Recently some substances which having blue-black toning effect upon image color, and can accelerate the process, were found. They are, for examples, 2-alkyl-1,3,4-oxadiazolin-5-thiones or 3-alkyl-benzoxazoline-2-thiones (Phot. Sci. & Eng. 4, 257-263 (1960)) and in patent-literatures other thiol compounds such as 5,5-dimethyl-4-thio-hydantoin, 5-benzildene-1,3-oxazolidine-4-on-2-thione or 5-methyl-3-mercapto-1,2,4-triazole.

These compounds usually called as blue-black toner, are not so effective with emulsions composed mainly silver chloride, and lose the toning effect by the presence of these silver complexing agents as thiosulfates, which make soluble complex with silver halide, in the developing solution.

Much efforts have been made by the inventors to obtain a useful blue black toners which can accelerate the rate of development even in the silver complex diffusion transfer processes which use a developer containing thiosulfates. It was found at first that 4-amino-1,2,4-triazoline-5-thione has a remarkable accelerating effect on the image formation in an image-receiving layer, yet unfortunately has little effect as a blue-black toner. After investigating a great number of compounds, two series of the derivatives of this compound having the following general formulas (A and B) were found to possess excellent properties not only to give dense-black or blue-black transfer images but also to accelerate the image formation in a silver complex diffusion transfer process;



wherein  $R_1$  represents a hydrogen atom or one of lower alkyl, aryl and aralkyl groups and  $R_2$  represents a lower alkyl group. Substances of B series are N-acyl derivatives of A.

Considerable differences are found between the characteristics of the above-mentioned two series of derivatives. All of the first mentioned A series show a remarkable development-accelerating effect, but a tone-modifying effect varies with the number of carbon atoms in  $R_1$ .

While the effect being influenced by changes of conditions such as concentrations of the agent, contents of thiosulfates, kinds of halogen in the silver halide grains, dimensions of grains in the emulsion, temperature, usually the tone-modifying effect tends to be enhanced initially with the increase of carbon atoms in  $R_1$  and after reaching maximum tends to fall off at a certain number of carbon atoms in  $R_1$  (see Example 2).

The derivatives of B series, on the other hand, show little developing retarding effect compared with the well-known blue-black toners, can hardly show any tendency to accelerate the process and rather tends to retard it with increase of the carbon atoms in  $R_1$  and  $R_2$ . These compounds, however, have very excellent blue-black toning or tone-modifying effects, which tends to be lower with the increase of carbon atoms in  $R_1$  and  $R_2$ .

So it is clear that some of the compounds of both series having lower alkyl, aryl or aralyl substituents, alone can be an excellent toner in themselves, compared with usual known compounds; but the above mentioned characteristics of the two series of compounds are mutually complemented and using both series of compounds in combination may result in high effects which cannot be obtained using the compound alone, and the compounds which have rather low utility when used alone can easily exhibit more excellent effects than any other known additives by being used jointly.

Any compounds of these two series can be used in combination with some of the known toning agents for the purpose of obtaining further practical merits.

The typical derivatives of A series include

4-amino-3-methyl-1,2,4-triazoline-5-thione,  
4-amino-3-ethyl-1,2,4-triazoline-5-thione,  
4-amino-3-propyl-1,2,4-triazoline-5-thione,  
4-amino-3-butyl-1,2,4-triazoline-5-thione,  
4-amino-3-p-tolyl-1,2,4-triazoline-5-thione,  
4-amino-3-p-methoxyphenyl-1,2,4-triazoline-5-thione,  
4-amino-3-p-chlorobenzyl-1,2,4-triazoline-5-thione, etc.

The typical derivatives of B series include

4-acetamide-1,2,4-triazoline-5-thione,  
4-acetamide-3-methyl-1,2,4-triazoline-5-thione,  
4-acetamide-3-ethyl-1,2,4-triazoline-5-thione,  
4-acetamide-3-propyl-1,2,4-triazoline-5-thione,  
4-acetamide-3-butyl-1,2,4-triazoline-5-thione,  
4-ethylamide-3-methyl-1,2,4-triazoline-5-thione,  
4-ethylamide-3-ethyl-1,2,4-triazoline-5-thione,  
4-ethylamide-3-propyl-1,2,4-triazoline-5-thione,  
3-methyl-4-pyropylamide-1,2,4-triazoline-5-thione,  
3-ethyl-4-propylamide-1,2,4-triazoline-5-thione,  
4-butylamide-3-methyl-1,2,4-triazoline-5-thione,  
4-acetamide-3-phenyl-1,2,4-triazoline-5-thione,  
4-acetamide-3-p-chlorophenyl-1,2,4-triazoline-5-thione,  
4-acetamide-3-p-tolyl-1,2,4-triazoline-5-thione,  
4-acetamide-3-benzyl-1,2,4-triazoline-5-thione,  
4-propylamide-3-p-chlorobenzyl-1,2,4-triazoline-5-thione,  
4-acetamide-3-phenethyl-1,2,4-triazoline-5-thione,  
4-acetamide-3-p-methoxybenzyl-1,2,4-triazoline-5-thione, etc.

They can be added in the developer solution, but usually it is favourable to introduce them into the receiving layer (or the over-layer upon it) or the sensitive layer (or the over-layer upon it), because the toner or toners in these layers diffuse out into the developer which are applied between the layers during the process.

The required concentration of the toner widely varies according to various factors involved in the system, such as temperature, contents of thiosulfate in the developer, etc. as mentioned above, but probably lies in a range between 0.01 to 10 g./l. in the developer and 0.01 to 0.1 g./m.<sup>2</sup> in the image-receiving layer or the light-sensitive layer, as a total sum of the agents used alone or in combination with similar compounds.

Compounds of this invention are soluble in an aqueous alkaline solution and are very stable in a solution of caustic alkalin. The properties are suitable to be added in a developer of the silver complex diffusion transfer system. The effects are not influenced very much by the temperature of developer, but it is favourable to carry out the development at a temperature between 15° C. and 35° C., considering the rate of diffusion of the silver complexes in the layer.

The derivatives of 4 - amino-1,2,4-triazoline-5-thione show a Tautomerism as follows:



The compounds of this invention can be prepared as schematically described below:



4-acetamido-3-ethyl - 1,2,4 - triazoline-5 - thione, for example, can be prepared as follows: 106 grams of thiocarbohydrazide and 222 grams of propionic acid are mixed 30 and heated for 9 hours at a temperature of 140° to 150° C. to yield 86 grams (60% of the theoretical amount) 35 4-amino-3-ethyl-1,2,4-triazoline - 5 - thione (M.P. 149° - 150° C.), whereupon 72 grams of the latter compound is dissolved in 100 ml. acetic anhydride and the solution is 40 heated for 3½ hours at a temperature of 90° to 95° C., then cooled and resulting crystals are dissolved in an aqueous solution of sodium hydroxide. Acidification of the alkaline solution to a pH value 5 by adding hydrochloric acid gives 35 grams of colourless crystals (M.P. 202°-203° C.). Other derivatives can also be prepared 45 in a similar manner with ease.

#### EXAMPLE 1

A light-sensitive material was prepared by coating a 45 paper support with a silver chloride-gelatin emulsion of low sensitivity.

An image-receiving material was prepared by coating a paper support with a suspension from the following coating composition:

50 Water—4 l.  
Gelatin—120 g.  
Polyvinylalcohol—60 g.  
3% solution of copolyvinyl-methylether-maleic anhydride in water (pH is adjusted to 6.0)—1 l.  
55 1% colloidal dispersion of cadmium sulfide in water—60 ml.

Coating weights of the suspension was adjusted to about 40 to 60 g./sq.m. And after drying precoating, a protective coating of 1.5% solution of sodium carboxymethyl-cellulose in water (about 30 g./m.<sup>2</sup>) was applied over the 60 coating.

A light-sensitive paper was exposed image-wise, while being in contact with an original to be reproduced, whereupon it was passed together with the above image-receiving 65 material through a developing bath of the following composition:

|                                            | G.  |
|--------------------------------------------|-----|
| Hydroquinone                               | 12  |
| 1-phenyl-3-pyrazolidone                    | 1   |
| 70 Anhydrous sodium sulfite                | 60  |
| Sodium hydroxide                           | 12  |
| Potassium bromide                          | 1.5 |
| Sodium thiosulfate                         | 10  |
| 4-amino-3-propyl-1,2,4 triazoline-5-thione | 0.3 |
| 75 Water up to 1 l.                        |     |

## 5

When leaving the developing bath, both materials are pressed together and then, after a contact period of one to five seconds, separated from each other. An image with completely dense black tone was obtained in the present image-receiving layer. When the same amounts of 4-amino-1,2,4-triazoline-5-thione was used instead of the above-mentioned 3-propyl derivative, the diffusion rate of the silver complex was so rapid as well, but the image-tone was rather brown and unfavourable. Without these compounds, 30 to 60 seconds of a contact period were needed to obtain an image of an unfavourably yellowish brown tone on the same image-receiving layer.

## EXAMPLE 2

The table below shows the colour-ratio, defined as the ratio of the reflection density measured at 400 m $\mu$  to that at 700 m $\mu$ , of a transferred image on an image-receiving material obtained by the diffusion transfer process using developers which consist of almost the same components described in Example 1 and using various toning agent of 4-amino-1,2,4-triazoline-5-thione derivatives. The image-tone is generally represented by the colour-ratio, and the image-tone was brown or brownish black when the colour-ratio was larger than two, and it was neutral black or blue-black when it was smaller than two on the contrary.

TABLE OF COLOUR-RATIO

|                      | R <sub>1</sub>                         |     |                  |                                |                                |                                |                                 |       |                                 |
|----------------------|----------------------------------------|-----|------------------|--------------------------------|--------------------------------|--------------------------------|---------------------------------|-------|---------------------------------|
|                      |                                        | H   | -CH <sub>3</sub> | -C <sub>2</sub> H <sub>5</sub> | -C <sub>3</sub> H <sub>7</sub> | -C <sub>4</sub> H <sub>9</sub> | -C <sub>5</sub> H <sub>11</sub> | -pH   | -C <sub>7</sub> H <sub>15</sub> |
| A-----               | -----                                  | 4.7 | 2.3              | 1.6                            | 1.5                            | 2.9                            | 4.4                             | ----- | 3.9                             |
| R <sub>2</sub> ----- | {B-----                                | 2.2 | 2.0              | 1.9                            | 2.2                            | 2.3                            | 2.8                             | ----- | 3.9                             |
|                      | {C <sub>2</sub> H <sub>5</sub> -----   | 0.9 | 1.2              | 1.4                            | 1.6                            | 2.2                            | 1.9                             | ----- | 2.5                             |
|                      | {B'-----                               | 2.7 | 2.7              | 3.0                            | 3.3                            | 3.6                            | 3.6                             | ----- | 3.8                             |
|                      | {C <sub>2</sub> H <sub>5</sub> Ph----- | 3.2 | 3.0              | 3.2                            | 3.6                            | 3.3                            | 3.1                             | ----- | 3.8                             |

NOTE.—Ph means a phenyl group.

The above table demonstrates the effect of carbon-numbers of substituents upon the image-tone, and clearly indicates that the derivatives of B' series have only poor effect, and they are excluded from our invention.

## EXAMPLE 3

0.01 gram 1-phenyl-5-mercaptop-1,2,3,4-tetrazole and 0.01 gram mercapto-benzothiazole were added per litre of the emulsion described in the Example 1. They are well known stabilizing agents.

An image-receiving material was also prepared by coating a paper support with a suspension of the coating composition described in the Example 1 (coating weight=40 to 60 g./m.<sup>2</sup>).

After drying there was applied over the coating a further solution of the following composition as a protective layer. (about 30 g./m.<sup>2</sup>)

Sodium carboxymethyl cellulose—10 g.

Addition product of triethanolamine and sulfur dioxide—2 g.

1% solution of 4-amino-3-ethyl-1,2,4-triazoline-5-thione in ethanol—5 ml.

1% solution of 4-propioamido-3-methyl-1,2,4-triazoline-5-thione in ethanol—5 ml.

Sodium thiosulfate—6 g.

Water up to 1 l.

In this case, no addition of bluish black toning agents of the invention to the developer were needed and sodium thiosulfate was favourably decreased, accordingly usual commercial developers for the silver-complex diffusion transfer process could be used.

An example of the developer had the composition as follows;

Water—1 l.

Hydroquinone—10 g.

## 6

1-phenyl-3-pyrazolidone—1 g.  
Anhydrous sodium sulfite—70 g.  
Sodium hydroxide—15 g.  
Sodium thiosulfate—4 g.  
Potassium bromide—2 g.

## EXAMPLE 4

The coating solution for the protective layer of the image-receiving material described in the Example 3 was further added to 5 ml. of 1% solution of 2-methyl-5-mercaptop-1,3,4-triazol, a well known toning agent, in ethanol, and the amount of 1% solution of 4-propion-amido-3-methyl-1,2,4-triazoline-5-thione in ethanol was reduced to 2 ml. Thus, the combination of two or more toning agents leads to a wide latitude for the processing conditions such as temperature, and also serves to the reduction of the cost of material.

It is often more favourable to add the second toning agents into the light-sensitive layer as in the case of the Example 3. But, when hydrazines or amines are incorporated as an accelerator, it is favourable to add a toning agent into the developer as in the case of the Example 1.

## EXAMPLE 5

On the surface of the film base made of 0.05 mm. thin

polyethylene terephthalate subbed already for the coating of photographic emulsion by the method well known in the art or by the method described in U.S. Pat. 3,214,274, an image receiving layer was coated (about 50 g./m.<sup>2</sup>) from the following coating composition:

Water—7 l.  
Gelatin—120 g.  
Polyvinylalcohol—120 g.  
50 Copolymer of vinyl methyl ether and maleic anhydride—40 g.  
Half amide of the above mentioned polymer—20 g.  
1% colloidal dispersion of cadmium chloride in water—80 ml.

55 Over the coating an inter-layer of the following composition was coated (about 30 g./m.<sup>2</sup>);

Polyvinyl pyrrolidone—30 g.  
Water—1 l.  
60 10% solution of polyacrylamide (in water)—100 ml.  
Decolourable dyestuff (brown colour)—2 g.  
5% solution of saponin (in water)—200 ml.

65 After drying, silver-chloro-bromide gelatin emulsion, of which about a half amount of gelatin was displaced by the same amount of carboxy-methyl-starch and also added with 0.02 g./l. of benzotriazole as stabilizer, was coated on the inter-layer and finally 2% solution of carboxy methyl-starch was over coated as a protective layer.

70 The photosensitive material thus produced was particularly suitable for retrievals of the drawings for industrial design or architecture from a micro-filmed positive, and also suitable for obtaining inter-diapositives of medium size from original drawings by direct camera-copying.

After exposure by camera or enlarger, the sensitive material was processed for 30 sec. to 1 min. in the transfer-developer of the following composition;

|                                                | G.   |
|------------------------------------------------|------|
| 1-phenyl-3-pyrazolidone                        | 1.0  |
| Sodium sulfite anhydrous                       | 75.0 |
| Hydroquinone                                   | 10.0 |
| Caustic soda                                   | 15.0 |
| Sodium thiosulfate                             | 30.0 |
| Potassium bromide                              | 2.0  |
| 4-amino-3-propyl-1,2,4-triazoline-5-thione     | 0.06 |
| 4-acetamido-3-methyl-1,2,4-triazoline-5-thione | 0.04 |
| Water up to 1 l.                               |      |

During processing, a negative image was produced in an upper light-sensitive layer and a positive image was transferred into the lower image-receiving layer by diffusion-transfer process at the same time, then the material was transferred to the washing bath, where the upper layer was dispersed into water by means of the inter-layer which may be easily disintegrated into solution, and there left a final positive image on the film base in a very short time.

As fixing is not necessary in this operation, after a short rinse, after the film is treated by an acidic methanol solution, it will be quickly dried to get a positive picture consisted of a dense black lines and dots on a transparent film base.

#### EXAMPLE 6

60 ml. of 1% solution of 4-amino-3-propyl-1,2,4-triazoline-5-thione in ethanol plus 40 ml. of 1% solution of 4-acetamido-3-methyl-1,2,4-triazoline-5-thione in ethanol were advantageously added to the coating solution for the image-receiving layer described in the Example 5, instead of being added into the developer. In contrast with this, benztriazole was added into the developer instead of being added into the photo sensitive emulsion, but the latter case was disadvantageous, considering the stability of the photo sensitive materials.

#### EXAMPLE 7

0.07 g. of 4-acetamide-3-ethyl-1,2,4-triazoline-5-thione per 1 l. of emulsion was contained in the sensitive layer of Example 1. The same image-receiving material as in Example was prepared. A positive densely black image was immediately formed on the image-receiving material using the usual developing solution for the silver complex diffusion transfer process.

#### EXAMPLE 8

A sensitive material was prepared by coating the support paper of 90 g./m.<sup>2</sup> with gelatino-silver halide emulsion in such a way that 1.30 g. of silver chloride was present per 1 m.<sup>2</sup> of the sensitive material. A sensitive sheet was produced by coating the following solution on said emulsion layer at the rate of 1 l./10 m.<sup>2</sup>.

PAM75 (trade name for polyacrylamide having a medium viscosity and produced by American Cyanamide Company)—10 g.

10% solution of saponin—10 cc.

4-amino-3-ethyl-1,2,4-triazoline-5-thione—0.08 g.

Water—1000 cc.

The image-receiving material was produced by coating the following solution on a support paper of 80 g./m.<sup>2</sup> at the rate of 35 g./m.<sup>2</sup>.

Gelatin—10 g.

Barium sulfate—350 g.

Cobalt sulfide—0.8 g.

Sodium thiosulfate—100 g.

1% ethanol solution of 1 - phenyl - 5 - mercapto-tetrazole—25 cc.  
Water—160 cc.

A positive densely black image was immediately formed on the image-receiving material using the treating solution of Example 3 as the developing solution.

What we claim is:

1. In a photographic silver complex diffusion transfer process, the improvement which comprises effecting development and diffusion in the presence of at least one 4-amino-1,2,4-triazoline-5-thione derivative of the general formula:



wherein

$\text{R}_1$  is a member selected from the group consisting of hydrogen, lower alkyl, aryl and aralkyl, and

$\text{X}$  is a member selected from the group consisting of  $\text{NH}_2$  and  $\text{NH}-\text{CO}-\text{R}_2$  wherein  $\text{R}_2$  is a lower alkyl group, said process immediately producing a densely black transfer image.

2. The improved photographic silver complex diffusion transfer process according to claim 1, in which 4-amino-1,2,4-triazoline-5-thione derivatives used are selected from the group consisting of 4-amino-3-ethyl-1,2,4-triazoline-5-thione, 4-amino-3-propyl-1,2,4-triazoline-5-thione, 4-ethylamide-3-ethyl-1,2,4-triazoline-5-thione and 4-ethylamide-3-propyl-1,2,4-triazoline-5-thione.

3. In a developer for immediately producing diffusion transfer images comprising a silver halide solvent and at least one developing agent,

the improvement wherein said developer contains at least one 4-amino-1,2,4-triazoline-5-thione derivative of the general formula:



wherein

$\text{R}_1$  is a member selected from the group consisting of hydrogen, lower alkyl, aryl and aralkyl,

$\text{X}$  is a member selected from the group consisting of  $\text{NH}_2$  and  $\text{NH}-\text{CO}-\text{R}_2$  wherein  $\text{R}_2$  is a lower alkyl group, wherein said transfer images possess a densely black image tone.

4. A silver complex diffusion transferring material containing at least one of the derivatives according to claim 3 in an image-receiving material.

5. A silver complex diffusion transferring material containing at least one of the derivatives according to claim 3 in a sensitive layer or a layer adjacent thereto.

#### References Cited

##### UNITED STATES PATENTS

- |           |        |                  |       |       |
|-----------|--------|------------------|-------|-------|
| 3,017,270 | 1/1962 | Tregillus et al. | ----- | 96—29 |
| 3,335,009 | 8/1967 | Rasch et al.     | ----- | 96—61 |
| 3,232,759 | 2/1966 | White et al.     | ----- | 96—29 |

#### OTHER REFERENCES

Hoggarth, J. Chemical Soc., 1952, pp. 4811—4817.

NORMAN G. TORCHIN, Primary Examiner

W. H. LOUIE, Jr., Assistant Examiner

70 U.S. Cl. X.R.

96—52